

[54] METHOD FOR COATING AN ARTICLE

[75] Inventor: Akihiro Ohkuma, Hirakata, Japan

[73] Assignee: Matsushita Electric Industrial Co., Ltd., Kadoma, Japan

[22] Filed: Jan. 22, 1974

[21] Appl. No.: 435,577

[52] U.S. Cl. .... 427/101; 427/277; 427/299; 427/331; 427/375; 427/430

[51] Int. Cl.<sup>2</sup> .... B05D 1/18; B05D 3/00

[58] Field of Search..... 117/49, 47 R, 119.2, 113, 117/54, 120, 201, 218, 47 A, 8; 29/613, 610; 338/308; 426/91, 101, 306; 427/101, 277, 299, 331, 375, 430

## [56] References Cited

## UNITED STATES PATENTS

|           |        |                     |             |
|-----------|--------|---------------------|-------------|
| 597,277   | 1/1898 | Fagg .....          | 117/119.2 X |
| 2,191,352 | 2/1940 | Oprean .....        | 426/91      |
| 2,427,417 | 9/1947 | Prickett .....      | 117/8 UX    |
| 2,976,188 | 3/1961 | Kohl .....          | 117/8 X     |
| 3,167,451 | 1/1965 | Tierman .....       | 117/47 R    |
| 3,200,471 | 8/1965 | Johnson et al. .... | 29/613 X    |
| 3,584,379 | 6/1971 | Loose .....         | 29/610      |
| 3,722,077 | 3/1973 | Armstrong .....     | 117/49 X    |
| 3,728,144 | 4/1973 | Van Poucke .....    | 117/119.2 X |
| 3,736,179 | 5/1973 | Gier et al. ....    | 117/113 X   |

3,773,579 11/1973 Michelson et al. .... 117/49 X

Primary Examiner—Harry J. Gwinnell  
Attorney, Agent, or Firm—Wenderoth, Lind & Ponack

## [57] ABSTRACT

A method for coating an article with a layer of coating material. The article is first cooled to a temperature lower than the freezing point of a chlorofluoro ethane. Then there is prepared a suspension of said chlorofluoro ethane as a suspending medium with coating particles of the coating material dispersed therein, the particles being insoluble in the chlorofluoro ethane. The suspension is kept at a temperature higher than the freezing point of chlorofluoro ethane, and the article is immersed in said suspension so as to form a frozen layer of the suspension on the surface of the article by freezing of the chlorofluoro ethane. The article is taken out of the suspension and the chlorofluoro ethane contained in the frozen layer is removed by heating the article at a temperature higher than the boiling point of the chlorofluoro ethane to leave a layer of particles on the article. The article is then further heated so that the particles remaining on the surface of the article form a layer of the coating material on the article.

8 Claims, 7 Drawing Figures





FIG. 1



FIG. 2



FIG. 3



FIG. 4a



FIG. 4b



FIG. 4c



FIG. 4d

**METHOD FOR COATING AN ARTICLE****BACKGROUND OF THE INVENTION**

This invention relates to a method for coating an article, and more especially to a method of cool dip coating of an article suitable for mass-production.

There have been known various methods of coating articles with a resin coating or a glass coating. Practically, for the resin coating, the most popular method is one in which a vehicle including coating resin material is applied to an article by spraying or dipping, and the thus applied coating is cured after being dried. Another method is one in which a powdered coating resin is adhered to a heated article and is cured. For the glass coating, the conventional method is brush coating or dipping. For both the resin coating and glass coating, there exist problems in that the coating applied according to the conventional methods has an irregular thickness from portion to portion over each body coated and has a rather small thickness. In addition, in case of coating electronic components, it is difficult in the conventional methods to prevent contamination of a portion of the lead wire of the component to be soldered to an electric circuit.

**OBJECTS AND BRIEF DESCRIPTION OF THE INVENTION**

It is an object of this invention to provide a method for coating articles with a thick coating of resin or glass having a uniform thickness.

Another object of this invention is to provide a method for coating with a coating of resin or glass having no pin-holes and bubbles therein.

A further object of this invention is to provide a method for coating articles which is particularly effective for mass-production.

A further object of this invention is to provide a method for coating electronic components having lead wires attached thereto in which the lead wires are not contaminated by the coating material.

These objects are achieved by a method for coating an article with coating particles comprising; cooling said article to a temperature lower than the freezing point of chlorofluoro ethane which is a non-solvent for said coating particles, said chlorofluoro ethane being the suspending medium for a suspension with said coating particles of said resin dispersed therein; immersing said article in said suspension so as to form a layer of said suspension on the surface of said article by freezing of said chlorofluoro ethane, said suspension being kept at a temperature higher than the freezing point of chlorofluoro ethane; taking said article out of said suspension; removing chlorofluoroethane contained in said frozen layer by heating said article at a temperature higher than the boiling point of chlorofluoro ethane; and forming a layer of said resin of the remained particles on the surface of said article by heating.

**BRIEF DESCRIPTION OF THE DRAWINGS**

These and other objects and the features of the invention will be apparent from a consideration of the following detailed description taken together with the accompanying drawings, wherein:

FIGS. 1 and 2 are schematic views of an apparatus for carrying out the coating method according to the present invention;

FIG. 3 is a graph showing the relation between the thickness of the coated layer on the article and the temperature of the cooled article.

FIGS. 4(a) to 4(d) are schematic views showing the process of coating an electronic component of an axial type according to the present invention.

**DETAILED DESCRIPTION OF THE PREFERRED EMBODIMENT**

- 10 According to the invention, particles of coating material such as resin or glass to be coated are dispersed in a suspending medium which is a non-solvent for these particles, and a suspension of the coating particles is formed. As the suspension is kept at a temperature higher than the freezing point of the non-solvent suspending medium, it is in a fluid state. Further, the viscosity of the suspension is set so as to be suitable for immersing the article to be coated in the suspension by controlling the concentration of the particles of resin dispersed therein. For the case of the resin coating, a preferable concentration of the particles is nearly 10 to 50 weight % with respect to the non-solvent suspending medium. At a concentration of more than 50 weight %, the fluidity of the suspension is decreased undesirably for immersing the article in the suspension. For the glass coating, a preferable concentration is higher than that for the resin coating because the specific gravity of the glass particles is higher than that of the resin particles.
- 20 The article to be coated is cooled to a temperature lower than the freezing point of the non-solvent suspending medium and immersed in the suspension. Then, due to freezing of the non-solvent, a frozen layer of the suspension is formed on the surface of the article. This frozen layer is a mixture of the non-solvent suspending medium and the coating particles. If the article is left in the suspension having the temperature higher than a freezing point of the non-solvent suspending medium, the formed layer will be melted in the suspension. Therefore, the article on the surface of which the frozen layer is formed is taken out of the suspension, and at once the article is heated so as to evaporate the non-solvent suspending medium and to form a resultant layer consisting of only the coating particles. Then, by further heating the coating particles are cured and there is formed a uniform layer on the article.
- 30 The coating method described above is useful for mass-production because of its simplicity, and the formed layer is characterized by having a rather large thickness and no pin-holes. Further, because of the cooling method, it is convenient to coat the article such as a film capacitor for which heating is undesirable so that coating thereof is difficult by the conventional method. Further, according to this method, an article of any shape such as a tubular article can be easily coated. Some articles having a complex shape are difficult to be coat the conventional methods such as spraying.
- 40 An operable material which can be used as the non-solvent suspending medium for the resin particles includes a chlorofluoro ethane system having a preferable freezing point near room temperature. When the freezing point is too low, there are the problems in that it is difficult and expensive to cool the article to be coated to a temperature lower than that freezing point. Further, as the article is apt to be wet due to the water content of the air, pin-holes are caused in the formed
- 45
- 50
- 55
- 60
- 65

layer. On the other hand, when the freezing point of the non-solvent suspending medium is too high, there is caused loss of the non-solvent due to heating of the suspension. Further, if the boiling point of the non-solvent becomes too high, the resin particles are melted before the non-solvent is evaporated fully and so the formed layer becomes uneven because it contains the non-solvent component therein. In addition, increasing the temperature of the suspension is undesirable because it decreases the pot life of the coating particles. Although there are various kinds of chlorofluoro ethanes, from the point of practical working operation for cooling the article and evaporating the non-solvent, the preferable ones are  $CCl_2FCCl_2F$  (designated by the international code 112),  $CCl_3CClF_2$  (112a) and  $CCl_2FCClF_2$  (113a) which have freezing points of  $23.5^{\circ}C$ ,  $40.6^{\circ}C$  and  $14^{\circ}C$ , respectively and have the boiling points of  $92.8^{\circ}C$ ,  $91.5^{\circ}C$  and  $45.7^{\circ}C$ , respectively. The temperature of the suspension is kept slightly higher than freezing point of the non-solvent suspending medium. When it is too high, the cooled article immersed therein is heated too quickly and the frozen layer of the suspension is not formed.

If the suspension has a low concentration of the coating particles, when the non-solvent is evaporated from the frozen layer of the suspension formed on the article during heating, there is sometimes caused slipping down of the layer of the remaining particles. In this case, it is effective to include a binder in the suspension. Then, the layer does not slip down but is transferred to the next curing process. In order to form a uniform layer, the binder should be soluble in the non-solvent suspending medium for the resin particle, particles with which the article is being coated. For the case of a resin coating, materials operable as a binder include polystyrene and denatured silicon resin. The latter dissolves epoxy resin, which is preferably used as the coating material for the method of the invention, well. The preferable concentration of the binder ranges 0.1 to 5.0 weight %. Too much binder has an undesirable influence on the properties of the resin particles and causes unevenness of the resultant layer.

Now, there will be described in more detail embodiments of the invention in the following examples.

#### EXAMPLE 1

Disk type resistors were coated with epoxy resin as described hereinafter referring to FIGS. 1 and 2. In FIG. 1, the disk type resistors designated by the reference numeral 1 were cooled to a temperature of nearly  $5^{\circ}C$  in a cooling room 2. Dried air was continuously fed into the cooling room 2 and an immersing room 3 from an inlet 4. The cooled resistors were transferred to the immersing room 3 past a heat shielding wall 5, and immersed in a suspension 6 contained in an immersing tank 9.

The suspension 6 was formed by particles of epoxy resin having the hereinafter described composition as the coating material and a mixture of 90 weight parts of 1,2-difluoro, 1,1,2,2-tetrachloro ethane ( $CCl_2FCCl_2F$ ) and 10 weight parts of 2,2-difluoro 1,1,1,2-tetrachloro ethane ( $CCl_3CClF_2$ ) which was a non-solvent for the particles. Such a mixture is available on the market under the trade name Daiflon S<sub>2</sub> (made by Daikin-kogyo Co., Japan), which has a freezing point of  $26^{\circ}C$  and a boiling point of  $91^{\circ}$  to  $93^{\circ}C$ . The composition of the epoxy resin is as follows:

|                      |                                                                           |
|----------------------|---------------------------------------------------------------------------|
| principal component: | BIS phenol-A type epoxy resin, Epikote 1007 (Shell Chem. Co. U.S.A.) 100g |
| 5 hardener:          | aromatic amine, 4,4' Diamino-Diphenyl Sulfone 3.5g                        |
| filler:              | SiO <sub>2</sub> 25g                                                      |
| lubricant:           | Stearic acid 1.0g                                                         |
| pigment:             | Fe <sub>2</sub> O <sub>3</sub> 11g                                        |

10 The composition has a melting point of  $100^{\circ}$  to  $119^{\circ}C$ . The concentration of the particles of epoxy resin in the suspension was 10 to 50 weight %. The temperature of the suspension was continuously kept nearly at  $30^{\circ}C$  by means of a heater 10 and a cooler 11. Further, the suspension was loosely stirred by a stirrer 12 so as to make the concentration of the particles in the suspension uniform. When the resistors were immersed in the suspension 6, the stirring was stopped. A frozen layer 7 was thus formed on each resistor.

15 After the resistors were immersed in the suspension for 5 seconds, the resistors were taken out therefrom. There was a frozen layer 13 of the suspension, i.e., the mixture of the particles of epoxy resin and the non-solvent suspending medium Daiflon S<sub>2</sub>, on the surface of each resistor. The resistors 1 taken out of the suspension were instantly transferred to the next step of the process. That is, the non-solvent was evaporated by heating the resistors in a drying room 14 shown in FIG. 2. Then, there was formed a layer 15 consisting of only the particles of epoxy resin:

20 The layer 15 may slip down if some vibration is applied to the resistor. Also, with a low concentration of the particles of epoxy resin in the suspension, there may be caused a similar problem. The slipping down of the layer 15 can be prevented by adding polystyrene in a concentration of 100 ppm to the suspension as a binder. Denatured silicon resin was also effective for preventing the slipping down of the layer 15.

25 The dried layer 15 was further heated at  $130^{\circ}C$ , the curing temperature for the epoxy resin, for 20 minutes, and then there was formed a cured layer 16. The thickness of the resultant layer was 1.0 to 1.2 mm.

30 The transferring of the resistors into and out of the rooms 2, 3 and 14 were carried out continuously by providing shutter mechanism. The vapor of the non-solvent in the drying room 14 was absorbed by a vacuum pump 17 and condensed by a cooler 18. The condensed vapor can be collected in a container 19. This is desirable for reducing the coating cost.

35 Usually, the thickness of the formed layer increases in accordance with an increase of temperature difference between the article to be coated and the suspension. FIG. 3 shows such a relation between the temperature of the article and the thickness of the resultant layer for the conditions indicated in the figure.

#### EXAMPLE 2

40 A suspension similar to that of Example 1 was used. The concentration of the particles of epoxy resin was 35 to 45 weight %, and the temperature of the suspension was kept at  $27^{\circ}$  to  $32^{\circ}C$ . Three resistors, of the axial of electronic component having two lead wires extending longitudinally from both ends, one 8 mm in diameter and 40 mm in length, 8 mm in diameter and 20 mm in length, and one 1.5 mm in diameter and 8 mm in length, were cooled to a temperature of  $-9^{\circ}$  to  $-15^{\circ}C$ , and immersed in the suspension 41 for 5 to 10

seconds to a depth such that 1.5 mm of one lead wire 44 above the upper end of the resistor body 42 was covered, as shown in FIG. 4(a). Then, the frozen layer 43 of the suspension was formed, as shown in FIG. 4(a) and FIG. 4(b), on the surface of the resistor body 42, the other lead wire 44' and the part of the lead wire 44, which were immersed in the suspension 41.

After the resistors were taken out of the suspension, a cutter 45 was pressed into the frozen layer formed on the lead wire 44' from a horizontal direction A, as shown in FIG. 4(c), so as to cut that layer, and then the cutter 45 was moved as while being held in the cutting position downwardly in the direction B sliding along the lead wire 44'. By this operation, the frozen layer 46 formed on the lead wire 44' was easily separated therefrom.

This process of pressing and moving the cutter was carried out while the formed frozen layer 43 was kept as it was. Even by this process, the layer 43 formed on the resistor body was not deformed. It was not necessary to cut around the complete circumference of the lead wire 44', and even by cutting only a part of the layer 46 it could be easily separated. Then, there remained only the desired portion the layer, i.e. on the resistor body and on a part of the lead wires.

Then, similarly to Example 1, the resistors were put in the drier at 120°C, wherein at first the non-solvent was evaporated and the surface of the particles of epoxy resin were partially melted, by which means slipping down of the layer due to heating could be prevented. In accordance with increase of temperature, the particles of epoxy resin melted and there was formed a uniform layer 47 as shown in FIG. 4(d). The thickness of the resultant layer was 0.6 to 1.0 mm.

### EXAMPLE 3

A suspension was made with the same non-solvent suspending medium as that of the example 1 and 30 weight % of particles of nylon 12, and 2 weight % of polystyrene were dissolved in the suspension as a binder. The same resistor as that of the example 2 was immersed in the suspension, and the frozen layer of the suspension was formed similarly. After separating the layer on the lead wire similarly to example 2, the remaining layer was cured by heating the resistor at 200°C. Then, there was formed a uniform layer of nylon 12.

### EXAMPLE 4

33 weight % of particles of polyvinyl chloride were dispersed in the same non-solvent suspending medium as that of example 1, and a cooled iron plate was immersed in the resultant suspension. The frozen layer of the suspension formed on the surface of the iron plate was cured at 120°C, and there was provided an iron plate coated a uniform layer of polyvinyl chloride.

### EXAMPLE 5

Wirewound resistors were coated with glass of having a low melting point by using suspension system having the following composition:

|                                |        |
|--------------------------------|--------|
| glass powder                   | 100g   |
| binder; ethylcellulose         | 2.15g  |
| non-solvent suspending medium; | 193.2g |
| Daiodon S <sub>2</sub>         |        |

The glass powder consisted of 88 weight % of PbO and 12 weight % of B<sub>2</sub>O<sub>3</sub> and had a 1.0μ average grain size. The suspension was kept at 27°C, and the wirewound resistors cooled at -12°C were immersed in the suspension, so that the frozen layer of the suspension was formed on the surface of the resistor. After taking the resistors out of the suspension, at first the non-solvent was evaporated, and then the resistors were kept at nearly 300°C for 30 minutes so that the binder was burned away completely. After that, the resistor was further heated at 350°C for 10 minutes to melt the glass powder completely. Then, the resistor was cooled to room temperature at a rate of 10°C/minute, and a uniform glass layer having no pin-holes and having a thickness of 0.8 mm was formed on the surface of the wirewound resistor.

What is claimed is:

1. A method for coating an article with a layer of coating material comprising:  
cooling said article to a temperature lower than the freezing point of a chlorofluoro ethane;  
providing a suspension of said chlorofluoro ethane as a suspending medium with coating particles of the coating material dispersed therein, the particles being insoluble in the chlorofluoro ethane;  
keeping said suspension at a temperature higher than the freezing point of chlorofluoro ethane;  
immersing said article in said suspension so as to form a frozen layer of said suspension on the surface of said article by freezing of said chlorofluoro ethane;  
taking said article out of said suspension;  
removing the chlorofluoro ethane contained in said frozen layer by heating said article at a temperature higher than the boiling point of said chlorofluoro ethane to leave a layer of particles on the article;  
and  
heating the article and the particles remaining on the surface of said article to form a layer of the coating material on the article.
2. A method as claimed in claim 1, wherein said chlorofluoro ethane is selected from the group consisting of CCl<sub>2</sub>FCCl<sub>2</sub>F, CCl<sub>3</sub>CClF<sub>2</sub> and CCl<sub>2</sub>FCClF<sub>2</sub>.
3. A method as claimed in claim 1, wherein said coating particles are particles of resin.
4. A method as claimed in claim 3, wherein said particles of resin are dispersed in said suspension in a concentration of 10 to 50 weight % relative to said chlorofluoro ethane.
5. A method as claimed in claim 3, wherein said suspension contains a binder which is soluble in chlorofluoro ethane in a concentration of 0.1 to 5.0 weight %, said binder being selected from the group consisting of polystyrene and denatured silicone resin.
6. A method as claimed in claim 1, wherein said coating particles are glass particles.
7. A method as claimed in claim 1, wherein said article is an electronic component.
8. A method as claimed in claim 7, wherein said electronic component is an axial type component having two lead wires extending longitudinally from both ends thereof, one of said two lead wires and the whole body of said electronic component being immersed in said suspension, including the step of cutting off the layer of said suspension formed on the surface of said immersed lead wire, after the step of taking said component out of said suspension.

\* \* \* \* \*